

## UNITED STATES PATENT OFFICE

1,982,812

## CONTACT MATERIAL

Charles V. Iredell, East Orange, N. J., assignor to  
 Westinghouse Lamp Company, a corporation of  
 Pennsylvania

No Drawing. Application September 2, 1931,  
 Serial No. 560,863

1 Claim. (Cl. 200—166)

This invention relates to electrical contacts and is more particularly directed to means of this character especially adapted for use in high duty electrical service devices, as for example, heavy relays, motor starters, circuit breakers, short circuit switches and the like.

Contact means heretofore commercially produced and employed in high duty electrical devices have not been entirely satisfactory because of their deficiencies in one or more of the electrical or physical characteristics essential to good contact means.

An object of this invention is to provide contact means especially adapted for use in high duty electrical devices.

Another object of my invention is to provide contact means, the constituents of which permit them to be readily manufactured at a minimum cost into units of substantially uniform and unvarying dimensions.

Briefly the invention is directed to a novel contact means comprising generally a composite body consisting chiefly of a highly refractory metal, such as tungsten, molybdenum or the like, and a materially lesser refractory metal of appreciably greater electrical conductivity, such as copper, silver, or the like, together with a relatively small proportion of a carbonaceous material, such as graphite.

In the course of my experimentations with the manufacture and use of high electrical duty contact means, I have found that by following the method hereinafter outlined and by utilizing from twenty to eighty per cent of the highly refractory metal and eighty to twenty per cent of the materially lesser refractory and appreciably higher electrically conductive metal, together with a suitable proportion of carbonaceous material, such as graphite, ranging from two tenths of one per cent to ten per cent of the entire metallic constituents, comparatively inexpensive and highly satisfactory heavy electrical duty contact means may be obtained.

Although, by following the general method hereinafter outlined, these materials may be combined in any desired ratio within the above specified limits, I will now describe one of the preferred specific embodiments of my invention together with the novel method of producing the same.

The preferred contact means comprises a composite body which by weight consists of forty parts of silver, sixty parts of molybdenum and from one half to four parts of graphite. The contact means of this composition produced in

the below described manner has been found to have excellent heavy electrical duty characteristics.

Among others, some of the more essential properties of my novel contact means are as follows: its composition is such that it may be manufactured at a minimum cost in units of substantially uniform and unvarying dimensions; it will not promote ionization of the air on circuit breaking; its contacting surface is highly wear resistant and is not readily pitted.

Besides having the aforementioned advantageous properties one of the salient advantages of my novel contact means is that the voltage drop across the contacts when in operative position is relatively low so that the temperature of the contact means per se is correspondingly low to aid in maintaining the ambient air in the atomic or molecular state rather than in an ionized state, thus aiding in quenching the arc when the circuit is broken at that station.

In order that this contact means may be manufactured in a simple and expeditious manner I may employ the following initial products:

40 parts by weight of silver powder, all passing 80 a 200 mesh screen. 60 parts by weight of molybdenum powder, all passing a 150 mesh screen .5 to 4 parts by weight of powdered graphite, all passing a 200 mesh screen.

Any suitably sized charge is made up with the above constituents present in specified proportions. This charge is conveyed into the working chamber of a ball mill of appropriate size and milled for about an hour. By this operation the constituents of the charge are intimately 90 mixed with each other and are further pulverized.

After the milling operation, the resulting thoroughly and intimately mixed powder is formed into units of the desired size and shape in any suitable manner, such as by subjecting the powdered mixture in an appropriate die to a pressure of about one to twelve tons per square inch.

The thus formed units are then heated to a predetermined temperature for a sufficient length of time so as to insure a complete bonding of the particles and to develop a unitary structure having the desirable high electrical duty characteristics essential to a contact means. These results may be attained by heating the pressed units in a hydrogen atmosphere to a temperature of about 980° C. to 1020° C. for a period of about ten to thirty minutes.

100

105

110

The effect of this heat treatment is to fuse the silver to such a degree that it fills the interstices between the molybdenum particles and between the molybdenum and graphite particles. 5 When operating under these conditions, most of the molybdenum, silver and graphite remains in their elemental form, with a small proportion of the silver and molybdenum alloying, and a small proportion of carbon uniting with the molybdenum to form a carbide.

10 The pressure and firing conditions may be varied depending on the degree of hardness desired in the final product. If at any time after firing, it is found that the hardness of the product is below that required, it may be raised to the desired limit by placing the product under suitable pressure.

15 In this manner there is obtained contact means which during their manufacture do not appreciably wear away the inner surface of the dies, thus maintaining at a minimum the operating and replacement costs of production.

The contact units so formed may be buffed or polished to any desired degree, if so desired, before mounting, but I have found that after a mere brushing operation they can be efficiently employed as high electrical duty contact means. 80 These units may be mounted in any convenient manner, as by means of stud bolts, to the appropriate contact supporting strip of a high electrical duty device.

Having shown and described a specific embodiment of my invention I do not desire to be limited thereto except in accordance with the appended claims.

What is claimed is:

An electrical contact including a composite unit comprising by weight about 60% molybdenum and 40% silver, the molybdenum and silver being uniformly distributed throughout substantially the entire mass, the molybdenum being in the form of individual particles and being surrounded by the silver. 90 95

CHARLES V. IREDELL.

25

100

30

105

35

110

40

115

45

120

50

125

55

130

60

135

65

140

70

145

75

150